

April 10, 1951

J. BRAMLEY

2,548,514

PROCESS OF PRODUCING SECONDARY-ELECTRON-EMITTING SURFACES

Filed Aug. 23, 1945



Witness:  
Ann H. Bachus

Inventor  
Jerry Bramley  
by ~~At~~ Stark Carlson and Son  
Attorneys.

## UNITED STATES PATENT OFFICE

2,548,514

## PROCESS OF PRODUCING SECONDARY-ELECTRON-EMITTING SURFACES

Jenny Bramley, Long Branch, N. J.

Application August 23, 1945, Serial No. 612,197

2 Claims. (Cl. 117—33.22)

1

My invention relates to processes of secondary-electron-emission.

The present subject matter has been divided and the apparatus claims appear in U. S. Patent 2,527,981, granted October 31, 1950, for Secondary-Electron-Emitter, on continuation-in-part application Serial No. 20,016, filed April 9, 1948. The species relating to the dielectric formed from the metallic base is contained in continuation-in-part application Serial No. 102,618, filed July 1, 1949 for Secondary-Electron-Emitting Surface.

The primary purpose of this invention is to obtain multiplication of secondary electrons much higher than that obtained in prior practice. This is accomplished in this invention by the proper construction of composite surfaces. One method is to interpose a layer of dielectric limited in thickness to 0.1 mm. and preferably not exceeding 0.03 mm. between a layer with at least moderately high secondary-electron-emissive properties (called henceforth the secondary-electron-emitting layer) on the one hand and a metallic base on the other hand. Suitable substances for the dielectric are oxides of aluminum, titanium, copper, or manganese or crystals of alkali halides. For the secondary-electron-emitting layer the following substances may be used: beryllium or an alloy or oxide thereof, magnesium (oxidized), aluminum, or an alloy or oxide thereof.

A further purpose relates to methods for increasing the emission of secondary electrons.

A further purpose is to obtain high multiplication in a secondary-electron-emitter without the undesirable features of photoelectric effect due to the presence of a photoelectric material, such as caesium, in the layer emitting secondary electrons.

A further purpose is to produce a secondary-electron-emitter of high multiplication while avoiding time lag between the start or stop of the primary current and the start or stop of high secondary electron emission.

A further purpose is to maintain close time coordination between a secondary-electron-emitter and the primary current by providing for the neutralization by electrons of the positive charge in the secondary-electron-emitting layer at a rate predetermined by the primary current. One method of accomplishing this is by separating the secondary-electron-emitting layer from the metallic base by an extremely thin layer of porous dielectric and by intruding particles of the secondary emission layer into the pores of the dielectric to assist in neutralizing the positive

2

charge by electrons. Another method consists in distributing particles of a non-oxidizable metal, e. g. gold, platinum, palladium, osmium, or iridium, which can act as impurity centers in the dielectric to assist in neutralizing the positive charge by electrons from the metallic base.

A further purpose is to enhance the secondary-electron-emission of magnesium oxide by baking it in vacuo at a temperature of 600° to 800° C.

10 A further purpose is to employ as a metallic base a metal such as aluminum, chromium, or copper, or an alloy thereof, which will form an adherent self-limiting oxide capable of acting as the dielectric, and to apply a secondary-electron-emitting layer over the oxide.

15 A further purpose is to decrease conductivity along the layer of the secondary-electron-emitter in the composite surface as by granulating the surface into a mosaic.

20 A further purpose is to oxidize a metallic base, such as aluminum, copper, or chromium, or an alloy thereof, or a corrosion resisting iron-chromium alloy, to form a dielectric, apply over it a secondary-electron-emitting layer, and expose 25 the layers to an elevated temperature for a short time to form a mosaic.

25 A further purpose is to use a metallic base of a metal forming an adherent oxide, such as aluminum, copper, or chromium, or an alloy thereof, 30 oxidize the surface of the base, thus forming a dielectric layer over the base; coat the surface with a non-uniform thin film of a non-oxidizable metal, such as gold, platinum, palladium, osmium, or iridium, which increases the conductivity of 35 the dielectric, deposit further a thin layer of the metal or alloy used in the metallic base, oxidize such thin layer, and over it apply a secondary-electron-emitting layer. If desired, several alternate layers of the non-oxidizable metal and the metal used in the metallic base may be applied, 40 and then the oxidation carried out.

45 A further purpose is to construct a secondary-electron-emitter from an alloy of a metal forming an oxide of suitable dielectric properties, such as aluminum, and a metal which is a good secondary-emitter, such as beryllium or magnesium, and to oxidize the surface of the alloy in such a way as to form a layer emitting secondary electrons over a dielectric layer. The alloy must be 50 free from any poisoning impurities, such as nickel.

A suitable method of bringing the secondary electron-emitter to the surface is hydrogen firing or burnishing under an inert liquid, such as benzene.

55 A further purpose is to reduce the electrical in-

put in a tube containing a thermionic cathode by using a small cathode requiring only a small current to heat it and obtaining high secondary electron emission from an auxiliary cathode, preferably in mesh form, constructed in accordance with this invention.

A further purpose is to employ an auxiliary cathode constructed in accordance with this invention to overcome prior art difficulties, such as grid emission due to grid contamination from oxide-coated cathodes, backfiring, and ignition of local spots. Since the primary thermionic current is only a small part of the total cathode emission, there is no necessity to use oxide-coated cathodes in tubes constructed according to this invention.

The drawings are useful in explaining the invention. They have been chosen for the purpose of clear illustration of the principles involved and to illustrate conventionally a few only of the possible embodiments of the invention. In the drawings like numerals refer to like parts.

Figures 1 to 4 and 3<sup>a</sup> are diagrammatic sections of composite surfaces useful in explaining the invention.

Figure 5 is a diagrammatic section of a vacuum tube embodying the invention.

Figure 6 is a diagrammatic perspective view of an auxiliary cathode.

One of the most important aspects of the invention relates to the production in electron tubes of extremely high emission of secondary electrons as a consequence of strong electrostatic fields initiated by bombardment with primary electrons of composite surfaces constructed in accordance with the invention. There must, of course, be a suitable source of primary electrons and these electrons should have a speed such that the ratio of the secondary electrons released from the secondary-electron-emitting element to the primary electrons of the beam impinging on the secondary-electron-emitting element is greater than unity.

The base, dielectric and secondary emitter are capable of being laid variously but always with the same resultant arrangement of layers and the same method of operation.

The metallic base 20 in Figure 1 may consist of any desired solid metallic material. The metallic base is covered by an extremely thin layer 21 of dielectric. Suitable dielectric materials are; aluminum oxide  $Al_2O_3$ , titanium oxide  $TiO_2$ , copper oxide, manganese oxide  $MnO$ , an inorganic crystalline phosphor, an inorganic vitreous phosphor, or an alkali halide, such as  $NaCl$ ,  $KCl$ ,  $LiCl$ . The alkali halides are inert and do not volatilize easily under the conditions of production of secondary emission.

The dielectric need not be a perfect insulator; it preferably will be a semi-conductor. The structure of the dielectric should preferably be very fine.

On the dielectric layer is deposited a thin layer 22 of a substance which is a good emitter of secondary electrons such as beryllium; beryllium oxide,  $BeO$ ; alloys of beryllium, particularly alloys of beryllium and copper; manganese (oxidized); oxidized magnesium alloys; aluminum; alloys predominantly aluminum, such as duralumin of any of the recognized varieties, especially aluminum alloy 17S ( $Al$  95%,  $Cu$  4%,  $Mg$  0.5%,  $Mn$  0.5%) or aluminum alloy 24S ( $Al$  93.8%,  $Cu$  4.2%,  $Mg$  1.5%,  $Mn$  0.5%), or the aluminum-magnesium (10% or 30%) alloy, or the aluminum-beryllium alloys, of which the one containing 30% beryllium

appears the most efficient. Among the above, the duralumins are unexpectedly effective out of all proportion to any characteristics previously suspected and greatly exceed pure aluminum in multiplication.

When this top or secondary-electron-emitting layer 22 is struck by primary electrons under suitable potential conditions, it emits a large number of secondary electrons and thus becomes positively charged and creates a strong electrostatic field between the metallic base and the dielectric layer 21. This electrostatic field pulls out electrons from the metallic base 20 through the dielectric thus producing a high multiplication of electrons.

The combined thickness of the dielectric layer and of the layer emitting secondary electrons must be very small, the desirable range being from 2 to 20 microns. While not in every case essential, this range of thickness should be used for best results.

One of the problems in the prior art has been to cause the secondary-electron emission to stop and start either in coincidence with the primary current or after only a brief and controllable time interval. Malter (Marconi) British Patent 481,170, September 7, 1936, uses caesium and is troubled by time lag between the start of the primary current and the start of the high secondary electron emission, as well as between the stopping of the primary current and the stopping of the secondary emission. (Malter, Physical Review, vol. 49, p. 478 and p. 879 (1936)). Furthermore, caesium deteriorates by volatilization in vacuo and causes objectionable photoelectric effects, which prohibit the use of the layer as an emitting surface in a photomultiplier tube.

In the present invention, the electron-emitting layer is non-photoelectric, and many advantages and avoidance of much difficulty are thereby obtained.

In order to prevent excessive time lag, the positive charge in the secondary-electron-emitting layer 22 must be neutralized by electrons from the dielectric 21 very quickly, but not quickly enough to interfere with extraction of secondary electrons by the electrostatic field. The extraction time has been estimated as about  $10^{-14}$  seconds.

The dielectric layer 21 may be deposited by spraying, settling, evaporation, or similar methods carried out at suitable temperatures, as well as by oxidation, as later explained. The secondary-electron-emitting layer can be deposited on the dielectric by dusting, evaporation, settling, or the like. I have discovered that in order to produce the high field necessary for electron extraction from the metallic base under the conditions of cold emission (about 1,000,000 volts per centimeter) the thickness of the dielectric layer is of importance. A voltage due to secondary-electron emission of more than a few thousand volts is not obtained in practice. For best results the thickness should be approximately 0.03 millimeter, and in any case the thickness of the layer should not exceed 0.1 millimeter. No limit on thinness is necessary provided the dielectric functions.

The invention is operative in its broader phases provided the metallic base, dielectric layer, and secondary-electron-emitting layer are as described, without further precautions to avoid time lag, but for best results special precautions to avoid time lag should be taken.

There are several ways, which I have discovered to overcome this trouble.

One method of overcoming time lag is to deposit the dielectric layer deliberately with perceptible porosity. This can be done, if the dielectric is applied by settling from a liquid, by controlling the fineness of grinding of the particles with a diameter of the order of ten microns have been found to be satisfactory in obtaining porosity. If difficulty is encountered with colloidal properties, an electrolyte may be added to cause dispersion and hence aid settling.

The porosity permits molecules of the secondary-electron-emitting layer at sufficiently high temperatures to penetrate the dielectric, thus assisting in preventing time lag by conducting electrons to the surface and neutralizing the positive charge. Figure 2 shows at 22' projections from the secondary-electron-emitting layer into openings at 21' in the dielectric.

An alternate method of eliminating time lag by improving the electron conductivity of the dielectric when bombarded by the primary beam is to incorporate a discontinuous film of a non-corrodible metal not more than a few molecular diameters thick which may act as an impurity center in the dielectric. Any one of the noble metals, such as gold, platinum, palladium, osmium, or iridium, can be used.

The thickness of the non-corrodible metal layer must not exceed four molecular diameters, and a thickness of two molecular diameters gives best results. The film must be discontinuous or a series of islands. This is readily obtained by depositing the film by evaporation at reduced pressure and elevated temperature, or by electrode sputtering (John Strong, *Procedures in Experimental Physics*, Prentice Hall, 1938), or other similar methods well known in the art. The thickness of the layer of non-corrodible metal can be judged by the color on the walls of the evaporator, as well known in the art.

On the discontinuous non-corrodible metal film is deposited another layer of dielectric of the same thickness limitation and other characteristics as the first layer, before the layer of secondary electron emitter is applied. The second layer of dielectric is applied so that the non-corrodible metal will not act as a collector of primary electrons but will form an interstitial impurity center for the dielectric.

Figure 3 shows the non-corrodible metal film, such as gold, at 23, and the second dielectric layer at 24.

As shown in Figure 3a, there may be several alternate layers of dielectric 24' and non-corrodible metal 23', provided the total dielectric thickness does not exceed the limit set of 0.1 mm.

As explained above, the field intensity, which produces cold emission from the base metal at the base-metal-dielectric interface, will fall too low if any individual dielectric layer is allowed to become thicker than about 0.1 mm.; preferably 0.03 mm. If for other reasons the dielectric layer must be thicker, this can be accomplished by several alternate layers of dielectric and secondary electron emitter, each dielectric layer of optimum thickness and not exceeding 0.1 mm. Thus in Figure 4, on the metallic base 20 I deposit a layer of dielectric 24 (porous or possibly with a discontinuous film of non-corrodible metal sandwiched between two parts of the dielectric layer) then follow with a layer of secondary electron emitter 25, then another dielectric layer 26

as above of optimum thickness, then another layer 27 of secondary electron emitter, and so on until the desired total thickness of dielectric has been used, the top layer consisting, of course, of secondary electron emitter.

Where the secondary-electron-emitter is beryllium, it has been successfully applied to the tube element by evaporation in vacuo from electrically heated tantalum spirals which serve as supports and heaters. It does not matter whether the beryllium is oxidized or not, since the metal and oxide are equally good as secondary emitters.

Where magnesium is used as a secondary-electron-emitter, the oxidation is essential, as the un-oxidized metal is not a good emitter. The metal will, however, oxidize rather readily in air. I have discovered that the effectiveness of magnesium (oxidized) as a secondary-electron-emitter is greatly improved by the step of baking in vacuo at a temperature of from 600° to 800° C. The reason for the improved results from the baking in vacuo is thought to be at least partly due to the migration of magnesium into surface portion of the dielectric, and the fact has been clearly demonstrated.

The surface should be granulated into a mosaic. This can be done by firing in a hydrogen atmosphere at a temperature above 600° C. and below the softening point of the metal to reduce impurities and roughen the surface. It is then oxidized by exposure to the air, avoiding contamination, as from oil on the fingers. The surface is then etched, as by an acid or alkali. The secondary-electron-emitting layer is then deposited on top. The granulation appears to assist by preventing too ready conductivity across the electron-emitting layer.

An alternate technique for producing the mosaic is to expose the composite surface (metallic base, oxide, and secondary-electron-emitting layer) abruptly and briefly to a temperature in the range from 600°-800° C. for aluminum and higher or lower depending on the melting point for the other metals and alloys mentioned. For best results the exposure should be limited to a few seconds in order to insure that the secondary-electron-emitting layer (for example beryllium) be in the form of a well separated mosaic. The mosaic structure increases the surface of the dielectric exposed to the primary beam and reduces conductivity in the plane parallel to the metallic base.

There is no exact temperature at which beading or mosaic formation occurs, but rather a range as set forth within which the phenomenon is evidenced. The extent of mosaic formation is influenced by such factors as oxide film thickness and heat capacity of the metallic base.

On the other hand a very satisfactory secondary-electron-emitter is produced by using an alloy predominantly consisting of a metal which forms an adherent oxide, such as aluminum, copper, or chromium, self limited to 50 Angstroms thickness, and containing a substantial amount and up to 30% (typically 10%) of a metal such as beryllium and/or magnesium which is an excellent secondary-electron-emitter, either as metal or oxide or both.

It will usually not be profitable to employ less than 1% of the preferred secondary-electron-emitting element in the alloy.

The alloy must be substantially free from poisoning ingredients such as nickel or, less importantly, cobalt. Aluminum has been found to

give best results for the predominant metal of the alloy.

The alloy should be treated to concentrate the preferred secondary-electron-emitting component at the surface by metal migration. This can be accomplished by firing for a few seconds in hydrogen at 600° to 800° C. or by burnishing under an inert organic liquid such as benzene, toluene, or xylene.

The method of bringing the preferred secondary-electron-emitter to the surface as described in Junker and Leitgeb U. S. Patent No. 2,254,805 may also be used. The alloy is then oxidized as by exposure to the air at ordinary temperature. A preferred method of oxidation in alloys predominantly consisting of aluminum is to immerse in an alkaline solution of an oxidizing agent, such as ferric hydrate, heated to about 115° C., for a few minutes, depending on the desired oxide thickness. In this way the resultant is first the alloy forming a base metal layer, then a mixture of oxides containing particles of the dominant metal and its oxide, and finally a secondary electron emitting layer consisting chiefly of BeO, MgO, or a mixture. The electron emitting properties of this combination are very high.

The composite surfaces just described may be utilized in several distinct types of apparatus, as will be evident from the following discussion.

For electron photo-multipliers such composite surfaces will be useful particularly for cathodes emitting-secondary-electrons under electron bombardment. As well known, metals whose surfaces are covered with alkali or alkaline earth metals have high emissive properties (Görlich U. S. Patent No. 2,317,754). By the features of the present invention set forth herein, the secondary emission is still further enhanced. As well known in the art, such electron photo-multipliers may serve various functions, some of which are shown by Slepian U. S. Patent No. 1,450,265 or Piore U. S. Patent No. 2,123,024.

Proper adjustment of the conductivity of the dielectric in the composite surface emitting secondary electrons under bombardment is contemplated.

Secondary-electron-emitters according to the invention may also be used to increase the efficiency of thermionic vacuum tubes or gaseous tubes such as diodes, triodes, thyratrons, and the like. The thermionic cathodes in present use require a relatively large electrical input in order to produce any appreciable current from cathode to anode. In accordance with this aspect of the invention, a large electron current can be produced by an auxiliary cathode constructed in accordance with any one of the methods for producing composite surfaces with enhanced secondary-electron-emission when this auxiliary cathode is bombarded by a weak primary electron current. Only a small power input is required to produce this weak primary electron current by thermionic emission.

An equally small additional power input is necessary to supply the voltage to the thermionic electrons to give them the energy required to produce very high secondary-electron-emission when they strike any one of the multiplier elements earlier described. The auxiliary cathode can be used in diodes, triodes, many grid tubes, thyratrons, and the like.

Figure 5 shows this device applied in a triode having an envelope 35 suitably evacuated and containing an anode 36, a grid 37, a cathode 38

and an auxiliary cathode 39 in the form of a mesh.

In electron multipliers, mesh secondary-electron-emitters have been developed by G. Weiss, U. S. Patent No. 2,243,178 dated May 27, 1941. Figure 5 is a diagrammatic view of the arrangement of tube elements in a triode with cylindrical electrodes. Figure 6 gives a schematic view of the cathode and auxiliary cathode. It will be evident that the auxiliary cathode 39' is supported at 41, and the cathode 38' is supported at 40. Other elements of the tube may take on any of their well known forms.

It will be evident that secondary-electron-emitters with high secondary-emission in combination with dielectrics and metallic bases may be used to advantage in other ways well known in the art.

The auxiliary cathode may be used to overcome certain disadvantages associated with the use of thermionic cathodes, such as back-firing, grid emission and ignition of local spots. In standard tubes with oxide-coated cathodes, some of the cathode material, such as barium, evaporates and settles on the grid. This contaminates the grid and gives rise to grid emission of electrons, disrupting the normal functioning of the tube.

Backfiring is conduction in the reverse direction (plate to cathode) when the plate potential is negative with respect to cathode. It is especially harmful in rectifiers. Backfiring is due to a deposit of electron-emitting substance on the plate. This cannot occur in the present invention since the secondary-electron-emitter does not evaporate at the operating temperature of the tube. However, in a very high frequency oscillator the plate may have a coating of secondary-electron-emission material to enhance the efficiency of the tube.

Local hot spots are due to uneven heating of the oxide coated cathode. They cause increased local evaporation and deterioration of the cathode. The cathode material used in my invention does not evaporate at the operating temperature of the tube, thus eliminating both difficulties.

The prior art, in seeking to overcome the difficulties, produced remedies not generally applicable. See Ct. Jobst, U. S. Patent 1,964,517, dated June 26, 1934; W. Espe, U. S. Patent 2,125,105, dated July 26, 1938; and H. Kolligs, U. S. Patent No. 2,147,447, dated February 14, 1939. These prior art devices do not make use of auxiliary cathodes coated with suitable emitters of secondary-electrons to eliminate all these difficulties.

As a result of investigation, the necessary features for a secondary-electron-emitter which will function efficiently as an auxiliary cathode have been determined. The following remarks apply particularly to eliminating grid contamination in high power triodes, but they apply equally well to eliminating this and other difficulties in various types of electron tubes. Oxide coated cathodes, now in vogue in high powered triodes, are used because they require the least energy input per unit thermionic output at saturation. These oxide coated cathodes cause grid contamination.

In accordance with the present invention, the primary thermionic current need be only a small fraction of the total cathode emission, the main part being supplied by secondary electrons from the auxiliary cathode.

Hence the oxide coated cathode need not be

used, and instead the cathode of the invention will desirably be uncoated, made of tungsten, thoriated tungsten or other material which will not evaporate at the operating temperature of the tube. The auxiliary cathode will have an outer layer of beryllium or other material as set forth above, which will have high secondary electron emission, but will not be effected either by melting or evaporating, at the operating temperature of the tube. To prepare the mesh described in Figures 5 and 6, the metallic base of the secondary cathode will best be aluminum or equivalent as explained above.

In view of my invention and disclosure variations and modifications to meet individual whim or particular need will doubtless become evident to others skilled in the art, to obtain all or part of the benefits of my invention without copying the structure shown, and I, therefore, claim all such insofar as they fall within the reasonable spirit and scope of my claims.

Having thus described my invention, what I claim as new and desire to secure by Letters Patent is:

1. The process of producing an improved multiplier element for an electron tube, which comprises depositing on a solid metallic base a di-

5 electric layer limited in thickness to values below 0.1 mm. and selected from the class consisting of oxides of aluminum, titanium, copper and manganese, depositing on the dielectric layer a secondary electron emitting layer which has a combined thickness with the dielectric layer of 2 to 20 microns, free from nickel, different from the dielectric layer, and selected from the group consisting of beryllium, beryllium oxide, magnesium oxide and aluminum, and heat treating the multiplier element at a temperature between 600° C. and the softening point of the metallic base.

10 2. The process according to claim 1, in which the dielectric layer is porous.

JENNY BRAMLEY.

#### REFERENCES CITED

The following references are of record in the file of this patent:

#### UNITED STATES PATENTS

| Number    | Name             | Date          |
|-----------|------------------|---------------|
| 2,075,377 | Varian           | Mar. 30, 1937 |
| 2,175,696 | Lederer          | Oct. 10, 1939 |
| 2,189,972 | Warnecke, et al. | Feb. 13, 1940 |
| 2,192,418 | Sommer           | Mar. 5, 1940  |
| 2,198,329 | Bruining, et al. | Apr. 23, 1940 |